

## UNITED STATES PATENT OFFICE

2,615,824

## METHOD AND COMPOSITION FOR IMPARTING WATER RESISTANCE TO TEXTILE MATERIAL

Francis W. Minor, Arlington, Va., Arnold M. Sookne, Washington, D. C., Milton Harris, Bethesda, Md., and Gray L. Pyle, Chicago, Ill., assignors, by mesne assignments, to the United States of America as represented by the Secretary of the Army

No Drawing. Application February 17, 1948,  
Serial No. 9,008

4 Claims. (Cl. 117—161)

1

This invention is concerned with the production of water-resistant materials. More particularly, it relates to a treatment of a normally water-nonresistant body, e. g. a textile, with a lower-alkyl-mono-substituted dichlorosilane or dibromosilane, whereby water-resistance is conferred upon such body.

It is known broadly to treat a glass, textile, or paper body with an organo-silicon halide in the vapor or liquid phase to make it water-repellent; see U. S. Patents No. 2,306,222, Patnode, and 2,412,470, Norton, and British Patent No. 575,675, British Thomson-Houston Company Limited.

The present invention is based on the discovery that certain lower-alkyl-monosubstituted dichalosilanes, particularly monomethyl dichlorosilane, confer greater water-resistance on water-nonresistant bodies than any organo-silicon halides heretofore used for that purpose. For instance, a textile treated with a silane contemplated by us, will absorb considerably less water upon prolonged exposure to rain (e. g. for 1 hour) than any other organo-silicon halide of the prior art.

It is generally assumed that the organo-silicon halide, upon application to the body to be treated, hydrolyzes by reacting with atmospheric moisture and/or with water previously absorbed in the body.



R being an organic radical, X a halogen atom, x ranging from 1 to 3, y from 0 to 2, and z from 1 to 3, the sum of  $x+y+z$  in the monomer being 4 (the valence of silicon). The hydrolysis product then is assumed to condense in situ to form a thin water-resistant silicone resin deposit upon the treated body:



It is also generally known to neutralize the hydrohalic acid formed during the hydrolysis by means of a base; see, for instance, U. S. Patent No. 2,306,222, page 2, col. 2, lines 16 to 21, and British Patent No. 575,675, page 3, lines 1 to 26. Selection of a proper neutralizing substance is important to avoid damage to the treated body, not only from the acid but from the neutralizing substance as well. In the course of our research we have discovered certain substances capable of controlling the hydrochloric or hydrobromic acid formed during hydrolysis, which substances are non-injurious even to a delicate fabric body and

2

contribute to high water-resistance values in the finished product.

Thus it is a principal object of our invention to provide a durably water-resistant body by treating a normally water-nonresistant body with a lower-alkyl-monosubstituted dichalosilane.

Another principal object of our invention is a water-resistant textile adapted for military and civilian uses when made into clothing, tentage, etc.

A further object of our invention is a novel organo-silicon halide treatment of a normally water-nonresistant body in the presence of a substance capable of controlling the acid formed during such treatment.

Still another object of our invention is a method for rendering textiles water-resistant, which method can be conveniently carried out in conventional textile treatment apparatus and which is readily taught to semi-skilled or even unskilled personnel.

Yet another object of our invention is a water-resistant textile body, whose water-resistance characteristics will not be appreciably impaired by repeated laundering or dry-cleaning.

Other objects and advantages of our invention will appear more fully in the following description thereof.

We have found that superior water-resistance properties are imparted to a normally water-nonresistant body by immersing it in a lower-alkyl-monosubstituted dichlorosilane or dibromosilane



dissolved in an inert solvent, i. e. a solvent which does not react with the silane. The alkyl substituent group may be methyl, ethyl or propyl.

40 Monomethyldichlorosilane ( $\text{CH}_3\text{SiHCl}_2$ ) is a substance well adapted for the purposes of our invention. Upon hydrolysis and subsequent condensation of the silane, the fabric or other body becomes water-resistant, which phenomenon is believed by us to be due to the formation of a silicone resin deposit having recurrent



groups; however, we do not wish to be understood to limit our invention to this particular theory. Suitable inert solvents are for instance 55 chlorinated hydrocarbons such as carbon tetra-

3

chloride, or liquid aliphatic or aromatic hydrocarbons, such as a petroleum solvent (e. g. "Varsol," a petroleum fraction boiling at about 150° C., made by Standard Oil Company) or benzene.

The hydrochloric or hydrobromic acid formed during hydrolysis may be removed by washing. However, we prefer to neutralize it first by means of a weakly alkaline substance such as sodium bicarbonate or an alkali metal salt of a fatty acid, e. g. sodium acetate or potassium acetate. Strong alkalies are unsuitable where used on a body liable to be attacked thereby. Beside the alkali metal salts of acetic acid, those of formic, propionic, and butyric acid are suitable to control the hydrogen halide. Surprisingly we have found further, that if the hydrolysis of the organo-silicon halide is carried out in the presence of epoxybutene



a highly water-resistant body results upon condensation of the silane, without strength loss from acid attack; we are at present unable to account for this surprising ability of the epoxy-butenes of controlling the mineral acid forming during hydrolysis.

Curing of the silane upon the body, which we believe to result in the formation of a silicone resin deposit, is effected by drying at room temperature, preferably followed by exposure to an elevated temperature. We have obtained good curing effects in the case of textiles by exposure to 105° C. to 150° C. for 15 minutes to 2 hours. The goods are washed prior to the drying and/or heating step, in order to remove the hydrohalic acid which forms as the by-product of the hydrolysis of the organo-silicon halide as well as the substance used for controlling the acid. The body should be clean prior to commencement of the treatment, as dirt unfavorably influences the chemistry of the reaction; thus a fabric should be thoroughly cleaned by washing or dry-cleaning prior to treatment.

Particularly favorable results are accomplished by treating a woolen fabric in accordance with our invention, as wool is an acid-resistant fiber; but cotton, paper and other bodies can be made water-resistant with our method.

In evaluating water-resistance of the bodies treated in accordance with our invention, we have utilized the "dynamic absorption test" described in par. 5b (1) of CCC-T-191a Supplement, October 8, 1945, to Federal Standard Stock Catalog, section IV (part 5), Supplement to Federal Specification for Textiles; General Specifications, Test Methods. This test measures the interfiber liquid absorption of a textile by simulating the effect of immersion in an agitated body of water, e. g. a river, and consists of tumbling a test specimen in a tumble jar filled one-third with water at 55 R. P. M. for a designated time interval (say 10, 20, 30 or 60 minutes), passing the specimen through a 60 lb. wringer twice (the first time without, and the second time between blotters), and weighing the specimen; the percentage of added-on weight of the specimen is its "dynamic absorption value." Naturally, the lower the "dynamic absorption value," the more water-resistant the fabric.

By subjecting an untreated sample of 18 oz. wool serge to "dynamic absorption" tests for various time intervals, we obtained the following results:

4

### DYNAMIC ABSORPTION VALUE PERCENT

| 10 Min. | 20 Min. | 30 Min. | 60 Min. |
|---------|---------|---------|---------|
| 32      | 46      | 49      | 55      |

The following examples of water-resistance imparting treatments of samples of the same 18 oz. wool serge in accordance with our invention will illustrate various ways of practicing our invention and the advantages obtained therefrom; however, we wish to be understood that the scope of our invention is not limited by any technical details recited in such examples as, for instance, strength of silane solution, exact length of immersion, duration and temperature of curing, etc., inasmuch as such details will be readily varied by those skilled in the art without departing from the spirit of our invention and without sacrificing any of the advantages gained thereby.

### Example 1

25 1 part by volume of monomethyl dichloro-  
silane is dissolved in 30 parts by volume of car-  
bon tetrachloride. A dry switch of serge is im-  
mersed in this solution for 2 to 4 seconds, the  
carbon tetrachloride is evaporated from the serge  
at room temperature, and the swatch is then  
30 treated with a .2% solution of sodium carbonate  
to neutralize hydrochloric acid forming as a hy-  
drolysis by-product. The swatch is now washed  
twice with water to remove the product of neu-  
tralization and any excess of sodium carbonate  
35 solution, and finally baked for two hours at 105°  
to 110° C. The resulting product showed an in-  
crease in dry weight of 1.1% over the untreated  
sample. Dynamic absorption values in percent  
were:

| 10 Min. | 20 Min. | 30 Min. | 60 Min. |
|---------|---------|---------|---------|
| 14      | 17      | 19      | 19      |

45 The fabric retains its water resistance even after repeated laundering:

### DYNAMIC ABSORPTION VALUE PERCENT

|                          | 10 Min. | 20 Min. | 30 Min. | 60 Min. |
|--------------------------|---------|---------|---------|---------|
| After 5 launderings..... | 19      | 20      | 24      | 27      |

Control tests substituting silanes of the prior art for waterproofing textiles, gave the following dynamic absorption values (prior to laundering):

|                        | 10 Min. | 20 Min. | 30 Min. | 60 Min. |
|------------------------|---------|---------|---------|---------|
| Methyl trichlorosilane | 26.5    | 34      | 34.5    | 50      |
| Diethyl dichlorosilane | 37.5    | 47      | 51      | 58.5    |
| Ethyl trichlorosilane  | 34      | 39      | 44      | 47      |

*Example 2:*

The treatment of Example 1 was repeated by substituting a solution of 1.5 part by volume of monomethyl dichlorosilane in 100 parts of carbon tetrachloride. Dynamic absorption values of the treated swatch were as follows:

| 10 Min. | 20 Min. | 30 Min. | 60 Min. |
|---------|---------|---------|---------|
| 18.5    | 21      | 22.5    | 26.5    |

## 5

Dynamic absorption values obtained from a swatch treated by substituting a solution of .5 part per volume of monomethyl dichlorosilane in 100 parts per volume of carbon tetrachloride were not as favorable as those obtained by using the preceding solutions, but still indicate appreciable water resistance:

| 10 Min. | 20 Min. | 30 Min. | 60 Min. |
|---------|---------|---------|---------|
| 25.0    | 30.5    | 35.2    | 43.4    |

## Example 3

A moist swatch of serge, containing 26% of water absorbed between its fibers, is briefly immersed in a solution of 1 part by volume of monomethyl dichlorosilane in 40 parts by volume of carbon tetrachloride. The solvent is evaporated in a fume hood, and the hydrochloric acid by-product of the hydrolysis is removed by two washings in a 2% solution of sodium acetate in water, followed by a 25 minute rinse in tap water, and baking for 2 hours at 110° C. The increase in dry weight is 0.9%, and dynamic absorption values in per cent as follows:

| 10 Min. | 20 Min. | 30 Min. | 60 Min. |
|---------|---------|---------|---------|
| 15      | 17      | 18      | 19      |

The treated fabric retains its water resistance after dry-cleaning, as shown by its "dynamic absorption values" after 1 hour's agitation in a hydrocarbon dry-cleaning fluid:

| 10 Min. | 20 Min. | 30 Min. | 60 Min. |
|---------|---------|---------|---------|
| 18      | 20      | 20      | 23      |

It is believed that best results with moistened fabric are achieved by placing it in "equilibrium" with the atmosphere, i. e. absorbing as much moisture as can be entirely absorbed within the fibers so that no liquid is sensibly present at the surface of the fabric. Thus the higher the temperature and relative humidity of the atmosphere, the more water can be held by the fabric without "sweating."

## Example 4

Dry swatches of serge were briefly immersed in a solution of one part by volume of monomethyl dichlorosilane in 25 parts by volume of carbon tetrachloride. The solvent is evaporated in a fume hood, and the hydrochloric acid by-product of the hydrolysis is removed by a 30 minute immersion in an aqueous solution of a weak base, as indicated in the table below. This is followed by a two hour rinse in water, a gentle squeezing out of excess water, and oven-curing for 2 hours at 105-110° C. Dynamic absorption values in per cent were as follows:

|                                                                                       | 10 Min. | 20 Min. | 30 Min. | 60 Min. |
|---------------------------------------------------------------------------------------|---------|---------|---------|---------|
| .2% sol. of Sodium carbonate                                                          | 15      | 17      | 19      | 22      |
| .2% sol. of Sodium hydroxide                                                          | 19      | 23      | 25      | 33      |
| .4% sol. of Sodium bicarbonate                                                        | 14      | 16      | 17      | 20      |
| Sol. of 2 ml. conc. $\text{NH}_4\text{OH}$ (28.5% $\text{NH}_3$ ) in 800 ml. of water | 16      | 18      | 20      | 23      |
| .2% sol. of Sodium acetate                                                            | 17      | 18      | 18      | 22      |

## 6

Thus, best water-resistance was accomplished by using sodium bicarbonate and sodium acetate solutions, followed by sodium carbonate and ammonium hydroxide. Least favorable is neutralization with sodium hydroxide solution.

## Example 5

Olive drab serge samples are pretreated by impregnation with a water solution of a salt of a weak acid, dried, and immersed in a solution of 1 part by volume of monomethyl dichlorosilane in 25 parts by volume of carbon tetrachloride. The solvent is evaporated and the (neutralized) hydrolysis byproducts removed by washing in water, and the swatches oven-dried at 105 to 110° C. for two hours. Dynamic absorption values were as follows:

| 20                                      | Impregnating Agent | 10 Min. | 20 Min. | 30 Min. | 60 Min. |
|-----------------------------------------|--------------------|---------|---------|---------|---------|
| Sodium carbonate (15%) <sup>1</sup>     |                    | 29      | 39      | 45      | 52      |
| Sodium bicarbonate (23.5%) <sup>1</sup> |                    | 19.5    | 25      | 29      | 36.5    |
| Sodium acetate (37%) <sup>1</sup>       |                    | 16      | 20      | 22.5    | 30      |

<sup>1</sup> Amount of salt deposited on swatch (percent per weight of swatch). Best water resistance was achieved with the sodium acetate impregnated swatches; free hydrochloric acid was absent, as could be determined from absence of discoloration.

## Example 6

Serge samples treated in accordance with Example 4 (.2 solution of sodium carbonate being the neutralizing agent up to the point of oven-curing), were cured in the following temperatures and for the following time intervals:

## DYNAMIC ABSORPTION VALUE PERCENT

| 40           | Temp.    | Time | 10 Min. | 20 Min. | 30 Min. | 60 Min. |
|--------------|----------|------|---------|---------|---------|---------|
| 105°-110° C. | 60 min.  |      | 18      | 21      | 23      | 27      |
| 105°-110° C. | 90 min.  |      | 16      | 20      | 20      | 23      |
| 150° C.      | 15 min.  |      | 17      | 18      | 20      | 23      |
| Room         | 2 months |      | 17      | 18.5    | 21.5    | 26.5    |

Water resistance achieved by curing at 105 to 110° C. for 90 minutes, and by curing at 150° C. for 15 minutes is thus substantially the same, and almost as good as obtained by curing for two hours at 105° to 110° C. in accordance with Example 4.

## Example 7

A moist swatch of serge in "equilibrium" with an atmosphere of 95% relative humidity was immersed for several minutes in a solution composed of 1.8% monomethyl dichlorosilane, 2.4% 3,4-epoxybutene-1, and 95.8% carbon tetrachloride. Heat developed, in the solution during the immersion, and fine bubbles were observed for 1 1/4 minutes. The carbon tetrachloride solvent was evaporated by suspension in a fume hood for 1 hour, and the swatch rinsed in tap water for 30 minutes and finally cured for 90 minutes at 110° C. The dried swatch was found to be free from hydrochloric acid and to have gained 7.2% of weight; its dynamic absorption values were:

|  | 10 Min. | 20 Min. | 30 Min. | 60 Min. |
|--|---------|---------|---------|---------|
|  | 19      | 25      | 28      | 36      |

7  
Example 8

Dry swatches of serge were treated with solutions of monomethyl dichlorosilane in various organic solvents (see table below), the solvent evaporated, the free hydrochloric acid (hydrolysis byproduct) neutralized with a sodium salt of a weak acid, rinsed, and oven-cured at 105-110° C. for 2 hours. Dynamic absorption values were:

| Solvent                                                                                 | Parts by vol. of solvent per 1 part by vol. of silane | 10 Min. | 20 Min. | 30 Min. | 60 Min. |
|-----------------------------------------------------------------------------------------|-------------------------------------------------------|---------|---------|---------|---------|
| "Skellysolve B" (a petroleum fraction boiling at about 80° C., manuf. by Shell Oil Co.) | 25                                                    | 20      | 24      | 26      | 32      |
| Petroleum "Ether" (a mixture of pentanes and hexanes boiling between 40° C. and 70° C.) | 25                                                    | 20      | 22      | 24      | 31      |
| Acetone                                                                                 | 33 $\frac{1}{3}$                                      | 26      | 35      | 43      | 50      |
| Ether                                                                                   | 33 $\frac{1}{3}$                                      | 23      | 30      | 37      | 45      |
| "Varsol" (a petroleum fraction manuf. by Standard Oil Co.) boiling at about 150° C.     | 33 $\frac{1}{3}$                                      | 14.5    | 18.5    | 21      | 27.5    |
| Benzene                                                                                 | 40                                                    | 16.5    | 18.0    | 19.6    | 21.1    |
| Moist Benzene                                                                           | 40                                                    | 16.2    | 17.8    | 18.8    | 20.8    |

The foregoing table shows that aliphatic and aromatic hydrocarbon solvents for the silane result in water resistance of the treated fabric to almost the same degree as carbon tetrachloride. Presence of a small amount of water in the solvent is apparently non-injurious, as shown by 30 the results accomplished with moist benzene. The comparatively poor water resistance with acetone or ether as the solvent indicates the inferiority of organic solvents containing oxygen in the molecule for the purposes of water-resistance imparting treatment in accordance with our invention.

The following examples show the results of water-resistance treatment in accordance with our invention on fabrics other than 18 oz. serge: 40

## Example 9

Various wool fabrics were subjected to a preliminary dry cleaning with carbon tetrachloride. The samples were then immersed briefly in a 45 solution of 1 part by volume of monomethyl dichlorosilane in 25 parts by volume of carbon tetrachloride. The hydrochloric acid formed as a byproduct of the resulting hydrolysis was neutralized with a water solution of a sodium salt of a weak acid, and the neutralization product was rinsed out. The samples were finally cured at 110° C. for about two hours. Dynamic absorption values of the treated samples were as follows (corresponding dynamic absorption values of untreated samples shown in parenthesis):

| Fabric           | 10 Min.    | 20 Min.      | 30 Min.      | 60 Min.   |
|------------------|------------|--------------|--------------|-----------|
| Woven felt       | 32 (133)   | 40.5 (134.5) | 43.5 (137.5) | 49 (136)  |
| Tropical Worsted | 19 (51)    | 21.5 (55)    | 23 (51)      | 26 (51)   |
| 32 oz. Melton    | 70.5 (135) | 68.5 (136)   | 93.5 (134)   | 103 (134) |

## Example 10

5 oz. poplin (a cotton fabric) was impregnated with sodium acetate ( $\text{CH}_3\text{COONa} \cdot 3\text{H}_2\text{O}$ ) from an aqueous solution so as to deposit 26% of sodium acetate per weight of sample. The sample was immersed in a solution of monomethyl dichlorosilane, the solvent was evaporated, the sample again immersed in an aqueous solution of sodium acetate, rinsed, and cured for two hours at 130° C. Dynamic absorption values of the treated 75

sample were (corresponding values of untreated poplin samples in parenthesis):

| 5 | 10 Min. | 20 Min. | 30 Min. | 60 Min. |
|---|---------|---------|---------|---------|
|   | 27 (45) | 30 (45) | 31 (46) | 34 (47) |

Another sample of 5 oz. poplin was immersed for several minutes in a solution composed of 1.8% monomethyl dichlorosilane, 2.4% 3,4-epoxybutene-1, and 95.8% carbon tetrachloride (see Example 7). The carbon tetrachloride solution was evaporated by suspension in a fume hood for one hour, the sample was washed in a water solution of sodium acetate, rinsed for 30 minutes in running tap water, and cured for 90 minutes at 110° C. Dynamic absorption values were (corresponding values of untreated sample in parenthesis):

| 10 Min. | 20 Min. | 30 Min. | 60 Min. |
|---------|---------|---------|---------|
| 26 (46) | 33 (48) | 34 (48) | 34 (48) |

Breaking strength of the treated sample was 81% of the untreated sample.

It will be seen from the foregoing description that by a water-resistance imparting treatment in accordance with the present invention, woolen textiles and other normally water-nonresistant bodies are converted into superior water resistant bodies. We are not able at this time to account for the reason why the choice of a lower-alkyl-monosubstituted dichloro- or dibromosilane results in waterproofing superior to results accomplished with fully substituted halosilanes (that is, silanes wherein all four valences of the silicon atom are satisfied by halogen and or-

ganic substituents); however, the results obtained by our method clearly show that such is the case.

We claim:

1. A method of imparting water resistance to a normally water-non-resistant textile material, comprising immersing said material into a solution in an inert solvent of a lower-monoalkyl-substituted dihalosilane selected from the group consisting of monoalkyl dichlorosilane and mono-alkyl dibromosilane and having not more than

three carbon atoms in its alkyl substituent chain and 3,4-epoxybutene-1, in the presence of moisture, whereby said substituted dihalosilane is hydrolyzed in situ and the hydrohalic acid formed as hydrolysis by-product is neutralized in situ, and exposing said material to an elevated temperature after its removal from said solution, whereby the hydrolyzed substituted silane is condensed in situ to a water resistant deposit.

2. A composition for imparting water-resistance to a normally water-non-resistant body, comprising a lower-alkyl-monosubstituted-silane selected from the group consisting of monoalkyl dichlorosilane and monoalkyl dibromosilane, and having not more than three carbon atoms in its alkyl substituent chain and 3,4-epoxybutene-1 in an inert solvent.

3. A composition for imparting water-resistance to a normally water-non-resistant body, comprising monomethyl dichlorosilane and 3,4-epoxybutene-1 in an inert solvent.

4. A method of imparting water resistance to normally water-non-resistant textile material, comprising immersing said material into a solution in an inert solvent of lower-monoalkyl substituted dihalosilane selected from the group consisting of monoalkyl dichlorosilane and monoalkyl dibromosilane and having not more than 3 carbon atoms in its alkyl substituent chain and 3,4-epoxybutene-1, in the presence of moisture, whereby said substituted dihalosilane is hydrolyzed in situ and at least part of the hydrohalic acid formed as hydrolysis by-product is neutralized in situ, removing said material and the hydrolyzed monoalkyl-substituted silane absorbed

5  
10  
15  
20  
25  
30  
35

therein from said solution, expelling the solvent absorbed in said material, neutralizing the remaining portion of the hydrohalic acid by-product of the hydrolysis remaining in said material with sodium acetate, and condensing the hydrolyzed substituted silane, which is absorbed by said material, in situ at an elevated temperature to a water-resistant deposit.

FRANCIS W. MINOR.  
ARNOLD M. SOOKNE.  
MILTON HARRIS.  
GRAY L. PYLE.

#### REFERENCES CITED

The following references are of record in the file of this patent:

#### UNITED STATES PATENTS

| Number    | Name    | Date           |
|-----------|---------|----------------|
| 2,306,222 | Patnode | Dec. 22, 1942  |
| 2,386,259 | Norton  | Oct. 9, 1945   |
| 2,412,470 | Norton  | Dec. 10, 1946  |
| 2,449,572 | Welsh   | Sept. 21, 1948 |
| 2,469,625 | Barry   | May 10, 1949   |

#### FOREIGN PATENTS

| Number  | Country       | Date          |
|---------|---------------|---------------|
| 418,230 | Great Britain | Oct. 22, 1934 |
| 116,470 | Australia     | Jan. 19, 1943 |

#### OTHER REFERENCES

Bennett, Concise Chemical & Technical Dictionary, Chemical Publishing Co., 1947, pp. XX